# EUROPEAN PATENT SPECIFICATION

(11) **EP 2 034 090 B1**
(45) Date of publication and mention of the grant of the patent: **22.10.2014**
(21) Application number: 08013659.1
(22) Date of filing: 30.07.2008
(51) Int. Cl.: D21C 9/00

(54) **Method and apparatus for semi-chemical pulping**
Verfahren und Vorrichtung zum semi-chemischen Aufschliessen
Procédé et appareil de semi-chimique réduction en pâte

(30) Priority: 07.08.2007 US 954446 P; 15.07.2008 US 173132
(43) Date of publication of application: 11.03.2009
(73) Proprietor: Andritz, Inc., Glens Falls, NY 12801 (US)
(72) Inventor: Stromberg, Bertil, Diamond Point, New York 12824 (US)
(74) Representative: HOFFMANN EITLE

(56) References cited:
- EP-A- 0 476 230
- WO-A-2005/116328
- US-A- 5 536 367
- US-A- 5 565 061
- US-A- 6 132 556
- US-A1- 2001 032 711
- US-B1- 6 277 240

## Description

### BACKGROUND AND SUMMARY OF THE INVENTION

The present invention generally relates to a method and system for making a semi-chemical pulp from lignocellulosic material.

Semi-chemical pulping processes are known. See, e.g., U.S. Patent No. 4,229,251 to Temler; U.S. Patent No. 4,073,678 to Hammond et al. Semi-chemical pulping processes have different requirements and different operating conditions than pulping processes involving Lo-Solids^{®} Cooking, such as those disclosed in U.S. Patent No. 5,489,363 to Marcoccia et al.

When making semi-chemical pulps (pulps with yields in the 65-85% yield range, typically used for production of corrugated medium used in box making), several different chemicals can be used, such as NaOH, Na₂CO₃, Na₂SO₃, kraft white liquor or kraft green liquor. In some instances, high temperatures (greater than 160°C) and short cooking times (an hour or less) may be used for making semi-chemical pulps.

In a stand alone semi-chemical pulp mill, NaOH, Na₂CO₃, and Na₂SO₃ may be used separately or in combination or subcombinations. These chemicals may be advantageous because they have a minimum smell and may be regenerated in relatively simple recovery systems typically used for kraft liquor, especially when NaOH and/or Na₂CO₃ are used. Each chemical or combination thereof may produce its own pulp characteristics from the different types of wood used (e.g., various types of hardwood). Accordingly, the particular combination or subcombination may be selected based on the individual criteria of a producer.

The simple process and relatively short retention time may make it impractical to try to perform multi-stage cooking processes.

When a semi-chemical production facility is operated in a kraft mill, it may make sense from a chemical make-up point of view to use green liquor. Green liquor is produced by combusting kraft black liquor and dissolving the resultant smelt into white liquor. White liquor generally includes a mixture of NaOH and Na₂S, and green liquor includes those chemicals in addition to the chemicals in the smelt resulting from the combustion of the black liquor. When using green liquor in a digester equipped with extraction screens, through which the spent liquor is extracted, quite often the extraction screens become coated with lignin.

This clogging or coating may be caused by lignin that has precipitated out of solution due to the lower pH at the end of the cook. The pH decrease may result from the consumption of carbonate ion (CO₃²⁻). As the solubility of lignin, which as been exposed to alkaline cooking conditions, decreases with lower pH, it may form a sticky tar-like substance, which coats the digester screens and may make them non-functional to the point that the digester has to be shut down and cleaned.

To combat this potential problem, many mills with this type of equipment may add substantial amounts of kraft white liquor with the green liquor (e.g., up to 20-30% of the total chemical charge), in order to keep the pH higher at the end of the cook. A higher pH at the beginning of the cook, however, may have a negative impact on the pulp yield and may make the operation less economical, as white liquor is more expensive to produce than green liquor.

US-A-2001/032711 describes a method and continuous digester system for pulp cooking with particular alkali profiles. The document is directed to chemical pulping and more specifically employs the "kraft" form of chemical pulping.

The same is true of EP-A-0 476 230, describing a process to improve continuous kraft pulping to produce a kraft pulp.

US-A-6,132,556 discloses a method of controlling pulp digester pressure via liquor extraction. A process to provide for the operational control of a kraft pulp digester is discussed.

Finally, the subject of US-B1-6,277,240 is also a kraft chemical pulping digester. The movement of the kraft chemically treated chips through the digester is improved while accomplishing sufficient extraction of the desired liquid from the digester.

### BRIEF DESCRIPTION OF THE INVENTION

The present invention relates to a method for inhibiting fouling of a black liquor extraction screen in a cooking vessel for semi-chemical pulping. The method comprises steps recited in claim 1.

Increasing the pH at the end of the cook may keep the screens cleaner for a longer period of time. The increased pH may be accomplished by adding white liquor or NaOH (or any other base) through a circulation and/or central pipe at the end of the cook.

The pH at or near the extraction screen(s) may be elevated when compared with the pH of liquor above the extraction screens. This, in turn, may increase the solubility of the lignin at or near the extraction screen(s).

In certain embodiments, the pH level is raised of a liquid at or near an extraction screen of a vessel in which semi-chemical pulping is performed. In certain embodiments, this may cause an increase in the solubility of lignin and may also decrease the tendency of an extraction screen to clog.

### BRIEF DESCRIPTION OF THE DRAWINGS

Figure 1 illustrates a digester in accordance with an embodiment of the present invention.
Figure 2 illustrates a digester in accordance with another embodiment of the present invention.

### DETAILED DESCRIPTION OF THE INVENTION

Figure 1 shows a portion of a semi-chemical pulping system 100 that includes a digester 110. The inputs to the digester 110 include a conduit 102, which generally contains at least green liquor and uncooked pulp comprising lignocellulosic material. Conduit 102 (or another conduit) may supply other chemicals, such as, for example, NaOH, Na₂CO₃, Na₂SO₃, and/or white liquor, to the digester 110. The inputs to the digester 110 also include conduit 108, which supplies white liquor, NaOH (and/or other bases), and/or other agents that may increase the solubility of lignin and/or decrease the likelihood of extraction screen clogging.

The pulp is cooked in digester 110, which contains various extraction screens. Though digester 110 may contain various extraction screens at different elevations, extraction screen 112 illustrates where the spent or used liquor (i.e., black liquor) is removed or extracted from the digester 110. Black liquor is extracted via conduit 114, which splits into conduit 116 and conduit 106. The flow content of conduit 116 is mixed with the flow content of conduit 108 (e.g., white liquor and/or NaOH) and recycled back into digester 110 via conduit 118. This recycle loop may facilitate the efficient extraction of lignin in the black liquor while perhaps reducing the amount of white liquor and/or NaOH required.

The end of conduit 118 is positioned at or near the extraction screen 112. The end of conduit 118 may deliver the contents of conduit 118 in a concentrated location at or near extraction screen 112 or may deliver the contents at or near substantially the entire surface of extraction screen 112 within the digester. Alternatively, the end of conduit 118 may be incorporated into the extraction screen 112. The distance from the addition point to the extraction screen may be such that the pH is increased across substantially the entire surface of the extraction screen so as to inhibit the adherence of lignin to the extraction screen.

FIGURE 2 shows a portion of another semi-chemical pulping system 200 that includes a digester 210. The inputs to the digester 210 include conduit 202, which generally contains at least green liquor and uncooked pulp. The conduit 202 may also supply other chemicals, such as, for example, NaOH, Na₂CO₃, Na₂SO₃, and/or white liquor. The inputs to the digester 210 also include liquor such as white liquor, NaOH (and/or other bases), and/or other agents through the conduit 208 that may increase the solubility of lignin and/or decrease the likelihood of extraction screen clogging.

The pulp is cooked in digester 210, which contains various extraction screens. Though digester 210 may contain various extraction screens at different elevations, the extraction screen 212 illustrates where the spent or used liquor (i.e., black liquor) is removed or extracted from the digester 210. In the illustrated embodiment, black liquor is extracted via conduit 206.

The liquor supply conduit 208 feeds into and/or through (as illustrated) a center pipe 220 of the digester. The end of liquor supply conduit 208 and/or center pipe 220 is positioned at or near extraction screen 212. The end of liquor supply conduit 208 and/or center pipe 220 may deliver the contents of the liquor supply conduit 208 and/or center pipe 220 in a concentrated location at or near extraction screen 212 or may deliver the contents at or near substantially the entire surface of extraction screen 212. Alternatively, the end of liquor supply conduit 208 and/or center pipe 220 may be incorporated into extraction screen 212. The distance from the addition point to the extraction screen may be such that the pH is increased across substantially the entire surface of the extraction screen so as to inhibit the adherence of lignin to the extraction screen.

In certain embodiments, furthermore, it may be possible to combine the recycle loop and center pipe in a single method or vessel.

While the invention has been described in connection with what is presently considered to be the most practical and preferred embodiment, it is to be understood that the invention is not to be limited to the disclosed embodiment, but on the contrary, is intended to cover various modifications and equivalent arrangements included within the scope of the appended claims.

## Claims

1. A method for inhibiting fouling of a black liquor extraction screen (112; 212) in a cooking vessel (110; 210) for semi-chemical pulping, the method comprising the steps of:
feeding lignocellulosic material and green liquor to the cooking vessel (110; 210) for semi-chemical pulping;
cooking the lignocellulosic material in the cooking vessel (110; 210) for semi-chemical pulping such that some or all lignin is separated from the lignocellulosic material, and wherein lignin is dissolved into a cooking liquor;
extracting via an extraction screen (112; 212) black liquor comprising dissolved lignin, wherein the black liquor is formed during the semi-chemical pulping process from the cooking vessel (110; 210); and
adding at least one of white liquor and a base to the cooking vessel (110; 210) at or near the extraction screen (112; 212), such that a pH at or near the extraction screen (112; 212) is elevated and lignin is inhibited from adhering to the extraction screen (112; 212).

2. The method of claim 1, wherein the base comprises NaOH.

3. The method of claim 1 or 2, wherein the step of feeding lignocellulosic material to the cooking vessel (110; 210) further comprises feeding at least one of NaOH, Na₂CO₃, Na₂SO₃ and white liquor to the cooking vessel (110; 210).

4. The method of any one of the preceding claims, wherein the step of adding white liquor and/or the base to the cooking vessel (110; 210) at or near the extraction screen (112; 212) occurs at the end of a cook when most lignin has been extracted from the lignocellulosic material.

5. The method of any one of the preceding claims, wherein the step of adding white liquor and/or the base to the cooking vessel (210) at or near the extraction screen (212) occurs using a central pipe (220) running through the center of the cooking vessel (210).

6. The method of any one of the preceding claims, wherein the step of adding white liquor and/or the base to the cooking vessel (110) at or near the extraction screen (112) occurs using a circulation loop (114, 116, 118) comprising a mixture of white liquor and/or NaOH and black liquor comprising dissolved lignin.

7. The method of any one of the preceding claims, wherein the step of adding white liquor and/or the base to the cooking vessel (110; 210) at or near the extraction screen (112; 212) creates a localized elevated pH at or near the extraction screen (112; 212) higher than the pH of the cooking liquor above the extraction screen (112; 212).

8. The method of any one of the preceding claims, wherein a pH of the cooking liquor at the end of the cook is 10 or higher, preferably between 10 and 13, and more preferably between 10 and 12.

## Patentansprüche

1. Verfahren zum Verhindern von Verschmutzung eines Schwarzlauge-Extraktionssiebs (112; 212) in einem Kochbehälter (110; 210) zum halbchemischen Aufschluss, wobei das Verfahren die Schritte aufweist:
Zuführen von Lignozellulosematerial und Grünlauge zu dem Kochbehälter (110; 210) zum halbchemischen Aufschluss;
Kochen des Lignozellulosematerials in dem Kochbehälter (110; 210) zum halbchemischen Aufschluss so, dass einiges oder alles Lignin aus dem Lignozellulosematerial abgetrennt wird und wobei Lignin in einer Kochlauge gelöst wird;
Extrahieren von Schwarzlauge, die das gelöstes Lignin enthält, mit einem Extraktionssieb (112; 212) aus dem Kochbehälter (110, 210), wobei die Schwarzlauge während des halbchemischen Aufschlussverfahren ausgebildet wird; und
Zugeben von zumindest einem aus Weißlauge und einer Base in den Kochbehälter (110; 210) an oder nahe dem Extraktionssieb (112; 212) so, dass ein pH-Wert an oder nahe dem Extraktionssieb (112; 212) angehoben wird und Lignin daran gehindert wird, an dem Extraktionssieb (112; 212) anzuhaften.

2. Verfahren nach Anspruch 1, wobei die Base NaOH aufweist.

3. Verfahren nach Anspruch 1 oder 2, wobei
der Schritt des Zuführens von Lignozellulosematerial zu dem Kochbehälter (110; 210) ferner Zuführen von zumindest einem aus NaOH, Na₂CO₃, Na₂SO₃ und Weißlauge zu dem Kochbehälter (110; 210), umfasst.

4. Verfahren nach einem der vorhergehenden Ansprüche, wobei
der Schritt des Zugebens von Weißlauge und/oder der Base zu dem Kochbehälter (110; 210) an oder nahe dem Extraktionssieb (112; 212) am Ende eines Kochens, wenn das meiste Lignin aus dem Lignozellulosematerial extrahiert wurde, stattfindet.

5. Verfahren nach einem der vorhergehenden Ansprüche, wobei
der Schritt des Zugebens von Weißlauge und/oder der Base zu dem Kochbehälter (210) an oder nahe dem Extraktionssieb (212) unter Verwendung einer zentralen Leitung (220), die durch das Zentrum des Kochbehälters (210) verläuft, stattfindet.

6. Verfahren nach einem der vorhergehenden Ansprüche, wobei
der Schritt des Zugebens von Weißlauge und/oder der Base zu dem Kochbehälter (110) an oder nahe dem Extraktionssieb (112) unter Verwendung einer Zirkulationsschleife (114, 116, 118), die eine Mischung aus Weißlauge und/oder NaOH und Schwarzlauge mit gelöstem Lignin aufweist, stattfindet.

7. Verfahren nach einem der vorhergehenden Ansprüche, wobei
der Schritt des Zugebens von Weißlauge und/oder der Base zu dem Kochbehälter (110; 210) an oder nahe dem Extraktionssieb (112; 212) einen lokal erhöhten pH-Wert erzeugt, der höher ist als der pH-Wert der Kochlauge über dem Extraktionssieb (112; 212).

8. Verfahren nach einem der vorhergehenden Ansprüche, wobei
ein pH-Wert der Kochlauge am Ende des Kochens 10 oder höher ist, vorzugsweise zwischen 10 und 13 und besonders bevorzugt zwischen 10 und 12 liegt.

## Revendications

1. Procédé d'inhibition d'encrassement d'un tamis d'extraction de liqueur noire (112 ; 212) dans une cuve de cuisson (110 ; 210) pour la fabrication de pâtes mi-chimiques, le procédé comprenant les étapes qui consistent :
à introduire un matériau lignocellulosique et une liqueur verte dans la cuve de cuisson (110 ; 210) pour la fabrication de pâtes mi-chimiques ;
à cuire le matériau lignocellulosique dans la cuve de cuisson (110 ; 210) pour la fabrication de pâtes mi-chimiques de sorte qu'une partie de la lignine ou toute la lignine soit séparée du matériau lignocellulosique, et dans lequel la lignine est dissoute dans une liqueur de cuisson ;
à extraire par l'intermédiaire d'un tamis d'extraction (112 ; 212) une liqueur noire comprenant de la lignine dissoute, dans lequel la liqueur noire est formée durant le processus de fabrication de pâtes mi-chimiques à partir de la cuve de cuisson (110 ; 210) ; et
à ajouter au moins l'une d'une liqueur blanche et d'une base à la cuve de cuisson (110 ; 210) au niveau du tamis d'extraction (112 ; 212) ou à proximité de celui-ci, de sorte qu'un pH au niveau du tamis d'extraction (112 ; 212) ou à proximité de celui-ci soit élevé et la lignine soit inhibée d'adhérer au tamis d'extraction (112 ; 212).

2. Procédé de la revendication 1, dans lequel la base comprend du NaOH.

3. Procédé de la revendication 1 ou 2, dans lequel l'étape qui consiste à introduire un matériau lignocellulosique dans la cuve de cuisson (110 ; 210) comprend en outre l'introduction d'au moins l'un du NaOH, du Na₂Co₃, du Na₂So₃ et de la liqueur blanche dans la cuve de cuisson (110 ; 210).

4. Procédé de l'une quelconque des revendications précédentes, dans lequel l'étape qui consiste à ajouter la liqueur blanche et/ou la base à la cuve de cuisson (110, 210) au niveau du tamis d'extraction (112 ; 212) ou à proximité de celui-ci se produit à la fin d'une cuisson lorsque la plupart de la lignine a été extraite du matériau lignocellulosique.

5. Procédé de l'une quelconque des revendications précédentes, dans lequel l'étape qui consiste à ajouter la liqueur blanche et/ou la base à la cuve de cuisson (210) au niveau du tamis d'extraction (212) ou à proximité de celui-ci se produit en utilisant un tuyau central (220) traversant le centre de la cuve de cuisson (210).

6. Procédé de l'une quelconque des revendications précédentes, dans lequel l'étape qui consiste à ajouter la liqueur blanche et/ou la base à la cuve de cuisson (110) au niveau du tamis d'extraction (112) ou à proximité de celui-ci se produit en utilisant une boucle de circulation (114, 116, 118) comprenant un mélange de la liqueur blanche et/ou du NaOH et de la liqueur noire comprenant de la lignine dissoute.

7. Procédé de l'une quelconque des revendications précédentes, dans lequel l'étape qui consiste à ajouter la liqueur blanche et/ou la base à la cuve de cuisson (110 ; 210) au niveau du tamis d'extraction (112 ; 212) ou à proximité de celui-ci crée un pH élevé localisé au niveau du tamis d'extraction (112 ; 212) ou à proximité de celui-ci plus élevé que le pH de la liqueur de cuisson au-dessus du tamis d'extraction (112 ; 212).

8. Procédé de l'une quelconque des revendications précédentes, dans lequel un pH de la liqueur de cuisson à la fin de la cuisson est supérieur ou égal à 10, de préférence compris entre 10 et 13, et de préférence encore compris entre 10 et 12.
